

## UNITED STATES PATENT OFFICE

2,141,593

## LUBRICATING OIL

Louis A. Clarke, Fishkill, and Charles C. Towne,  
Poughkeepsie, N. Y., assignors to The Texas  
Company, New York, N. Y., a corporation of  
Delaware

No Drawing. Application August 27, 1934,  
Serial No. 741,724

3 Claims. (Cl. 87-9)

This invention relates to the manufacture of synthetic lubricating oils, and particularly to synthetic lubricating oils of improved character having an increased viscosity index, and to synthetic oils applicable for blending with mineral lubricating oils to improve the character thereof.

In the production of high grade lubricating oils, it is well known that a relatively small change in the viscosity of the oil between temperatures of say 100° F. and 210° F., is desirable. In other words, it is advantageous for the oil to have a relatively flat viscosity-temperature curve, which means that the oil has a high viscosity index as defined by Dean and Davis in their article in Chemical and Metallurgical Engineering, vol. 36, page 618. Improvement in lubricating oils has heretofore been accomplished by refining, as by the use of selective solvents which are effective in extracting or separating naphthenic constituents from paraffinic constituents, thereby producing a resulting raffinate of increased viscosity index. This procedure involves expensive processing, and results in a reduced yield of finished oil.

The advantage of low pour point of a lubricating oil has long been recognized. Paraffin base and Mid-Continent lubricating oils have been subjected to dewaxing in order to reduce the pour point thereof. However, substantially complete removal of wax from such oils results in a lowering in viscosity index.

The present invention relates to the increase in viscosity index of naphthene base or paraffin base lubricating oils, which may or may not have been solvent refined as a primary step, by the addition thereto of a material which is active to increase the viscosity index without objectionably affecting other desirable properties thereof. More particularly, the present invention relates to the production of an improved lubricating oil of this type having increased viscosity index, by the addition thereto of a controlled proportion of a hydrogenated condensation product of an alkyl halide with an aromatic hydrocarbon. The invention also contemplates the preparation of synthetic lubricating oils by hydrogenation of the condensation product of an alkyl halide with an aromatic hydrocarbon.

In accordance with the present invention, the alkyl halide and the aromatic hydrocarbon are condensed to produce a viscous synthetic oil of lubricating character. Various types of alkyl halides can be used, including halides of normally gaseous olefines, such for example as ethylene chloride and propylene chloride, and also other aliphatic hydrocarbon halides. The dihalides of

the lower or normally gaseous olefines are particularly effective in this reaction.

Of the aromatic hydrocarbons, benzene and its homologues, such for example as toluene, mesitylene, tertiary butyl benzene, tertiary amyl benzene, normal butyl benzene, secondary butyl benzene, and the like may be employed. Likewise, halogenated derivatives of benzene and its homologues, such as chlorbenzene, are satisfactory.

The condensation is effected in the presence of a catalyst of the Friedel-Craft type, such as anhydrous halides of aluminum, iron, boron, manganese, nickel, zinc, antimony, cadmium, tin and the like. Very satisfactory results are secured with anhydrous aluminum chloride. With proper control of the proportions of the ingredients and the condensation reaction, a viscous synthetic lubricating oil may be produced. The condensation product may be allowed to stand and stratify into an upper oily layer and a lower sludge layer, which are then separated by decantation. The upper oily layer is preferably distilled to remove lower boiling liquids including unreacted chemicals, to obtain as a residue a viscous synthetic oil of lubricating character. This oil is then hydrogenated in accordance with well known hydrogenation practice, as by heating in the presence of hydrogen under pressure, and with or without a hydrogenation catalyst. A resulting synthetic oil of high viscosity index, which may be in excess of 100, is thereby obtained. This oil itself is useful as a lubricating oil. Or, it may be blended with a petroleum lubricating oil in controlled proportions, to thereby increase the viscosity index of the petroleum lubricating oil. For example, proportions of from about 1% to 25% of the hydrogenated synthetic oil may be added to a naphthene base or paraffin base petroleum lubricating oil to materially increase the viscosity index of the latter. However, the proportions of the blend may vary widely, and higher proportions of the synthetic oil up to about 50% or more may be employed. But for economical reasons the lower percentages range mentioned is preferred.

As a specific example of the present invention, the following is given:

1000 g. ethylene chloride were mixed with 1580 g. of benzene in the presence of 125 g. of anhydrous aluminum chloride. The mix was warmed gently with agitation to about 36° C., when reaction set in which continued without further application of heat until a temperature of 45° C. was attained. Further heating of the mix to 60° C. caused additional reaction to set

in. The reaction product was then allowed to stand over night, whereupon it stratified into an upper oily layer and a lower sludge layer, which were then separated. The upper layer was subjected to distillation, and a cut boiling between 250°-300° C. was removed. A residue of a synthetic oil of golden color remained. This oil had a viscosity index of 80, having a Saybolt viscosity at 100° F. of 174 and at 210° F. of 44. 10 The oil also had a high specific gravity of 1.03 and a low pour test of -25° F. When this oil is subjected to hydrogenation, by passing through a heating coil with hydrogen gas at a temperature of around 600° F. and under a pressure of 15 approximately 3000 lbs. per square inch, and passed over a hydrogenation catalyst such as nickel, a further reaction occurs with the production of a more saturated oil of lubricating character having a still higher viscosity index, 20 generally in excess of 100, and lower Conradson carbon. When the resulting hydrogenated oil is blended with a naphthene base oil, as in the proportion of about 25%, an increase in viscosity index of the order of about 30-50 points is effected. 25 Similarly, a blend of about 25% of this synthetic oil with a paraffin base petroleum lubricating oil results in an increase in viscosity index of the latter of about 20-30 points.

A satisfactory product may also be prepared 30 from the lower sludge layer. For example, a green oil having a viscosity index in excess of 100 was obtained from the sludge layer in the example mentioned above. This oil had a specific gravity of 1.04, a Saybolt viscosity at 100° F. of 403 and at 210° F. of 60, and a pour test of -20° F. When this oil is subjected to hydrogenation in the manner specified above, a still higher viscosity index lubricating oil is obtained which is very satisfactory for blending with a petroleum 40 lubricating oil in the manner described above.

Obviously many modifications and variations of the invention, as hereinbefore set forth, may be made without departing from the spirit and scope thereof, and therefore only such limitations should be imposed as are indicated in the appended claims.

We claim:

1. The method in the manufacture of a synthetic lubricating oil of high viscosity index and 50 other desirable properties, which comprises condensing about five parts by weight of ethylene chloride with about eight parts by weight of benzene in the presence of a Friedel-Craft catalyst of the character of anhydrous aluminum chloride to produce an oily condensation product, 5

separating the oily condensation product from sludge and removing lower boiling constituents therefrom to obtain a synthetic oil within the lubricating oil boiling range having a viscosity index of about 80 or above, and then hydrogenating the obtained oily product within the lubricating oil boiling range to produce a synthetic lubricating oil having a viscosity index in excess of 100. 10

2. The method in the manufacture of a synthetic lubricating oil of high viscosity index and other desirable properties, which comprises condensing about five parts by weight of ethylene chloride with about eight parts by weight of benzene in the presence of a Friedel-Craft catalyst of the type of anhydrous aluminum chloride to produce an oily condensation product, allowing the condensation product to stand to stratify into an upper oily layer and a lower sludge layer, separating the layers, removing lower boiling liquids from the upper layer to obtain a residue of a viscous oil within the lubricating oil boiling range having a viscosity index of about 80 or over, and then hydrogenating the viscous oil so obtained to produce a synthetic lubricating oil 30 having a viscosity index of over 100. 25

3. The method in the manufacture of a synthetic lubricating oil of high viscosity index and other desirable properties, which comprises condensing about five parts of ethylene chloride with 35 about eight parts of benzene in the presence of a Friedel-Craft catalyst of the character of anhydrous aluminum chloride to produce an oily condensation product, allowing the condensation product to stand to stratify into an upper oily 40 layer and a lower sludge layer, separating the layers, recovering a viscous oil within the lubricating oil boiling range from the lower sludge layer having a viscosity index in excess of about 100, and then hydrogenating the recovered viscous oil to produce a synthetic lubricating oil having a viscosity index substantially in excess of 100. 45

LOUIS A. CLARKE.  
CHARLES C. TOWNE. 50